

# UNITED STATES PATENT OFFICE.

KARL KREKELER AND PAUL KRAIS, OF ELBERFELD, GERMANY, ASSIGNORS  
TO THE FARBNFABRIKEN, VORMALS FR. BAYER & CO., OF SAME PLACE.

## BLUE DYE.

SPECIFICATION forming part of Letters Patent No. 518,458, dated April 17, 1894.

Application filed May 9, 1893. Serial No. 473,593. (Specimens.)

To all whom it may concern:

Be it known that we, KARL KREKELER and PAUL KRAIS, chemists, doctors of philosophy, and assignors to the FARBNFABRIKEN, VORMALS FR. BAYER & CO., of Elberfeld, subjects of the Emperor of Germany, residing at Elberfeld, Prussia, Germany, have invented a new and useful Improvement in the Manufacture of new Blue Coloring-Matter; and we do hereby declare the following to be a full and exact description of the invention.

Our invention relates to the manufacture of a blue coloring-matter produced by the reaction of the nitroso compound of diethylanilin hydrochlorate with gallamic acid.

In carrying out our invention practically we proceed as follows: Ten (10) kilos, by weight, of gallamic acid and fifteen kilos, by weight, of nitrosodiethylanilin hydrochlorate are mixed with ten kilos, by weight, of alcohol and then boiled, until a sample taken out from the reaction mixture dissolves in hot water with a clear blue color. The melt is then poured into one hundred kilos, by weight, of water and five kilos, by weight, of hydrochloric acid of 20° Baume are added. After some time the coloring-matter crystallizes in greenish needles which are filtered off and dried. The coloring-matter thus obtained has the following formula:



It forms greenish bright-crystals, soluble in cold water with difficulty, easily soluble in hot water with blue color. Concentrated sulfuric

acid dissolves the dye-stuff with blue color, which is changed into red on adding water; hydrochloric acid (20° Baumé) dissolves it with 50 red color. The coloring-matter is difficultly soluble in hot alcohol, almost insoluble in cold alcohol. The coloring-matter dyes wool mordanted with chromium salts from blue to bluish-violet shades of great clearness, cotton 55 mordanted with chromium salts in bluish-violet shades.

We are aware of the patent to Geigy, No. 410,733, of September 10, 1889, and do not claim the body therein described. It is essentially different in its application and dyeing qualities from the body of this application. The dyestuff described by Geigy is nearly insoluble in water, and is not capable of dyeing wool. The product of our application is easily soluble in water, and can be employed in dyeing without the addition of sodium bisulphite and with other dyestuffs. It can also be used in dyeing wool.

Having thus described our invention, what we claim, and desire to secure by Letters Patent, is—

1. The process above described for producing blue coloring-matter by the reaction of nitrosodiethylanilin hydrochlorate and gallamic acid in the presence of solvents as for example alcohol or acetic acid.

2. As a new article of manufacture the coloring-matter having the formula:



and which is easily soluble in hot water with

a clear blue color, soluble in concentrated sulphuric acid with the same color, which color turns into red on the addition of water, soluble in hydrochloric acid with red color and dyeing wool and cotton mordanted with chromium salts from blue to bluish-violet, substantially as described.

5 In testimony whereof we have signed our

names in the presence of two subscribing witnesses.

KARL KREKELER.  
PAUL KRAIS.

Witnesses:

WILLIAM ESSENWEIN,  
RUDOLPH FRICKE.

Correction in Letters Patent No. 518,458.

It is hereby certified that in Letters Patent No. 518,458, granted April 17, 1894, upon the application of Karl Krekeler and Paul Krais, of Elberfeld, Germany, for an improvement in "Blue Dyes," an error appears in the printed specification requiring the following correction, viz: In line 75, page 1, the word "nitrosodiethyanilin" should read *nitrosodiethylanilin*; and that the said Letters Patent should be read with this correction therein that the same may conform to the record of the case in the Patent Office.

Signed, countersigned, and sealed this 24th day of April, A. D. 1894.

[SEAL.]

JNO. M. REYNOLDS,  
*Assistant Secretary of the Interior.*

Countersigned:

JOHN S. SEYMOUR,  
*Commissioner of Patents.*